

3,551,158

PHOTOGRAPHIC SILVER HALIDE EMULSIONS  
WITH INCREASED SENSITIVITY

Harald Huckstadt, Cologne, Stammheim, August Randolph, Leverkusen, Wilhelm Saleck, Schildgen-Bergendorf-Gladbach, and Erwin Ranz, Leverkusen, Germany, assignors to Agfa-Gevaert Aktiengesellschaft, Leverkusen, Germany, a corporation of Germany  
No Drawing. Filed Dec. 20, 1966, Ser. No. 603,168  
Claims priority, application Germany, Dec. 28, 1965,

A 51,190

Int. Cl. G03c 1/28

U.S. CL. 96—107

5 Claims

## ABSTRACT OF THE DISCLOSURE

Photographic silver halide emulsions having their sensitivity increased by the combination of a polyethylene oxide sensitizer and a sulfonium salt



wherein:

R=a branched or unbranched alkyl or alkenyl radical containing up to 6 carbon atoms which may be interrupted by hetero atoms and substituted by at least one hydroxyl, carboxyl or epoxy group;

Z=an alkylene radical having up to 18 carbon atoms that can be substituted with at least one hydroxyl, carboxyl or epoxy group, and can be interrupted by a hetero atom such as at least one oxygen atom, or aralkylene; and

X=an anion.

The present invention relates to photographic silver halide emulsions chemically sensitized by the addition of heterocyclic sulfur compounds.

A number of methods have been described for improving the sensitivity of photographic silver halide emulsions other than by optical or spectral sensitization with sensitizing dyes incorporated in the emulsion. The incorporation of such dyes in the emulsion increases the optical or spectral range of sensitivity, and for this reason such dyes are commonly referred to as optical or spectral sensitizing dyes. Contrary to optical or spectral sensitizers the so-called chemical sensitizers are believed to react with silver halide to form, on the surface of the silver halide grain, sensitivity specks the chemical nature of which depends on the kind of the chemical sensitizer. The sensitivity of silver halide emulsions can be increased by chemical ripening or after-ripening during the preparation of the emulsion, by either prolonging the ripening time or by the addition of suitable substances such as compounds of noble metals or thiosulfate or other sulfur compounds. According to another method customarily employed the sensitivity of a photographic emulsion can be increased by the addition of development accelerators or chemical sensitizers to the emulsion, usually when it is completely ripened.

Suitable development accelerators are, for example, compounds containing onium groups (for example, quaternary ammonium or phosphonium and ternary sulfonium salts) and polyalkylene oxides and derivatives of polyalkylene oxides.

The process of chemical sensitization, however, reaches a limit beyond which further addition of sensitizing compounds or of prolonged digestion in the presence of a sensitizer, merely increases the undesired fog of the photographic emulsions.

In particular with respect to polyalkylene oxide sensitizers, many attempts have been made to increase the sensitizing action by modifying the chemical structure or by using them in combination with other compounds. However, in practice, none of these compounds completely meet the requirements as regards producing a satisfactory increase in sensitivity without concomitant increases in fog or poor keeping qualities.

The object of the present invention is to provide new chemical sensitizers which do not suffer the above disadvantages. Another object is to provide photographic silver halide emulsions having increased sensitivity and satisfactory keeping qualities.

We now have found the sensitivity of the silver halide emulsion chemically sensitized with polyethylene oxide or derivatives thereof can be further increased by the addition of an aliphatic or araliphatic sulfonium salt, the aliphatic radicals of which are substituted by hydroxyl, carboxyl or epoxy groups.

20 The sulfonium salts correspond to the following formulae:



wherein:

R=a branched or unbranched alkyl or alkenyl radical containing up to 6 C-atoms, which may be interrupted by hetero atoms, in particular oxygen and which is substituted by at least one hydroxyl, carboxyl or epoxy group;

Z=(1) an alkylene radical having up to 18 C-atoms, preferably up to 6 C-atoms, which alkylene radical may be substituted by at least one hydroxyl, carboxyl or epoxy group or which may be interrupted by hetero atoms, in particular at least one ether oxygen atom to give, for instance, ethylene ether or polyethylene ether groupings, or (2) aralkylene such as xylylene, and

35 X=any anion, for example, halide ions, such as chloride or bromide, perchlorate, paratoluenesulfonate or methanesulfonate ions.

The above mentioned groupings may, of course, carry further substituents provided that they neither impair the increase in the sensitivity which the compounds of the present invention provide nor have any adverse effects on the photographic properties of the emulsions. The following compounds have proved to be especially suitable:









- (C) a condensation product of amidophosphoric acid with polyethylene glycols and  
 (D) a quaternation product of tertiary polyamines with bifunctional polyalkylene oxides.

with a sensitivity increasing amount of a disulfonium salt 5 having the formula



wherein:

R=a branched or unbranched alkyl or alkenyl radical containing up to 6 carbon atoms and substituted by at least one hydroxyl, carboxyl or epoxy group;

Z—an alkylene radical having up to 18 carbon atoms that can be substituted with at least one hydroxyl, carboxyl or epoxy group, and can be interrupted by at least one oxygen atom, or aralkylene; and

X—an anion.

2. The combination of claim 1 wherein R represents 20 a hydroxyl substituted ethyl group.

3. The combination of claim 1 in which the cation of the sulfonium salt has the formula



4. The combination of claim 1 in which the cation of the sulfonium salt has the formula



10 5. The combination of claim 1 in which the cation of the sulfonium salt has the formula



#### References Cited

#### UNITED STATES PATENTS

2,848,330 8/1958 Chechak et al. \_\_\_\_\_ 96—108X

25 NORMAN G. TORCHIN, Primary Examiner

R. E. FICHTER, Assistant Examiner